

June 16, 1931.

W. S. BOHLMAN

1,809,826

PROCESS OF ELECTRODEPOSITING CHROMIUM

Filed Sept. 6, 1927

Fig. 1.



Fig. 2.



INVENTOR  
Walter S. Bohlman  
BY  
Gustav Thompson  
ATTORNEY

## UNITED STATES PATENT OFFICE

WALTER S. BOHLMAN, OF ATLANTIC CITY, NEW JERSEY, ASSIGNOR TO CHROMIUM CORPORATION OF AMERICA, OF NEW YORK, N. Y., A CORPORATION OF DELAWARE

## PROCESS OF ELECTRODEPOSITING CHROMIUM

Application filed September 6, 1927. Serial No. 217,597.

This invention relates to chromium plating, and aims to provide improvements therein.

The present invention provides a method of chromium plating particularly adapted for effecting such plating on areas which by the ordinary methods present unusual difficulties. It is particularly adapted for plating on the underside of articles, in recesses, 10 pockets, corners and the like, and on the inside of pipes, and particularly pipe having irregular axial shapes.

Chromium plating is accompanied by a considerable evolution of hydrogen gas in the area in which the metal is deposited, and where this gas accumulates or is trapped, as for example on the under side of articles, in pockets and recesses, and in pipe, plating may be interfered with or prevented following the ordinary methods of plating.

According to the present invention, I apply the solution to limited areas at a time, in the form of a stream, with lateral contact of the solution with the atmosphere near the zone of plating in such manner that, when the current is acting the gas generated in the plated area has lateral egress to the atmosphere.

Several modes of procedure in carrying out the process are illustrated in the accompanying drawings, wherein:

Figure 1 illustrates a mode of procedure in plating the inner sides of a large vessel, and

Fig. 2 illustrates a mode of procedure in plating the inside of a pipe having a bend therein.

Referring to Fig. 1, a plating solution is forced or projected in suitable manner, as from a metallic nozzle 10, against the portion 12 of a surface to be plated, such surface being here shown as the inner wall at the underside of a large vessel 13. The metallic nozzle 10 is conveniently covered with a rubber or other insulating covering 14 to protect the operator from shock and to avoid short circuits being formed between the nozzle and metallic objects with which it may come into contact. The stream of solution is conveniently forced through the nozzle 10 by pump

15, a suitable hose connection 17 being provided between the nozzle and the pump. The pump may draw the solution from any suitable supply. There is here shown a pan 19 beneath the nozzle for catching the solution falling back from the surface of the vessel 13, and this solution may flow off from the pan to any suitable receptacle through the pipe 21. The vessel 13 is made cathode by connecting it with the negative side of a source of current, as indicated at 25, and the nozzle 10 is made anode by connecting it with the positive side of the source of current supply, as indicated at 27.

The nozzle is moved to successive portions of the surface of the article to be plated, and the plating of a large area effected successively in this way.

The solution used is preferably a concentrated chromic acid solution, containing a catalyst, such for example as disclosed in the Fink Patent No. 1,581,188, granted April 20, 1926.

The electric current makes contact with the solution through the metallic nozzle 10, and flows through the stream of solution to the surface of the cathode article against which the stream strikes. The current effects the reduction of chromic acid and the deposit of the chromium, and also effects the release of hydrogen at the cathode. As the stream of solution is in contact with the atmosphere, the hydrogen gas has a ready means of egress from the plating zone, and hence even when plating is done on the underside of articles, in recesses, corners, pockets and the like, it has a ready means of egress from the stream to the atmosphere at the side of the stream, and thus avoids a condition where the hydrogen would accumulate and thereby retard or prevent the plating.

The stream may be divided into a plurality of streams and thereby provide air spaces for the escape of gas throughout the area against which the plurality of streams as a whole is directed.

With this method of plating it is difficult to estimate the area covered by the stream and over which plating is taking place. The current density must therefore in most cases

- be obtained by experiment. I may indicate that I use considerably higher voltages than used in ordinary chromium plating, ordinarily connecting the nozzle to a 100 to 120-volt
- 5 D. C. circuit. Using a one-sixteenth inch nozzle placed four inches from a surface, I obtain plating with an ammeter reading of one-half ampere.
- The proper current density for plating is 10 readily obtained by moving the nozzle closer to or further away from the cathode surface, until the desired plate is observed, and the current density during plating is regulated in like manner.
- 15 It is known that there is a co-relation between quantity of catalyst in the solution, current density and temperature, and with a known solution as regards concentration of chromic acid and catalyst content, an adjustment of the temperature is effected by having regard to the temperature of the article being plated, the heating effect of the current, and the temperature of the solution supplied to the nozzle. If the article is large and at 20 room temperature or below, a proper temperature in the zone of plating is effected by having the temperature of the solution considerably higher than the estimated temperature at which it is desired to effect plating
- 25 30 —say for example a plating temperature of 35 to 40° C. The solution projected from the nozzle should have a higher temperature than such estimated temperature, and in practice the solution issuing from the nozzle has a temperature very nearly corresponding to boiling temperature. The heating effect of the current is very great, and ordinarily the heating of the stream is obtained from the heating effect of the current the 35 solution supplied to the nozzle being ordinarily unheated. The supplying of the nozzle with cold or unheated solution has the advantage that higher current densities can be used than are ordinarily used in tank plating.
- 40 45 The heat generated in the stream of solution between the nozzle and cathode is not stored or accumulated in a body of solution in the zone of plating, but passes off with the solution falling back from the cathode, and therefore the stream can carry a higher current density than could be used in plating a surface of equal area immersed in a plating solution in a tank.
- 50 A second mode of practising the invention is illustrated in Fig. 2. The article to be plated is a pipe 30, and is shown as having a right-angle bend therein. With such a pipe it would be difficult to fit an inside anode, and also difficult to prevent an objectionable accumulation of hydrogen. According to my process, a pipe 32 having a suitable nozzle 34 on one end, is inserted into the pipe 30, and a stream of liquid projected laterally against the inner side of the pipe 30, the pipe 32 and nozzle 34 being moved lengthwise of the pipe
- 55 60 65 70 75 80 85 90 95 100 105 110 115 120 125 130
- 30 to coat successive areas. The pipe 32 may be made flexible to follow the contour of irregularly shaped pipes, and the pipe 32 and nozzle 34 may be inserted first into the pipe to be plated at one end and then into the pipe to be plated at the other end. Suitable insulated supports 36, 37 for the pipe 32 may be provided if desired.
- The nozzle 34 is conveniently of a nature to project a disk-shaped or radiating stream, as here shown. Pipe 32 is made anode, as by connecting a conductor 38 thereto, and the pipe 30 is made cathode as by connecting a conductor 40 thereto, the conductors 38 and 40 being connected respectively to the plus and minus side of a source of current. Plating solution is continuously supplied to the pipe 32 during plating, in any suitable manner.
- The disk-shaped stream of plating solution communicates with the atmosphere on either side, so that there is a ready means of egress of the hydrogen evolved during the process, from the zone of plating, and in this manner accumulation of hydrogen which would interfere with the plating, is avoided.
- The invention is applicable to other plating solutions wherein considerable volumes of gas are released during plating in the cathode area.
- The invention may be practiced in many other modes of procedure than those herein specifically illustrated and described.
- What is claimed is:—
1. A method of electrodepositing chromium comprising projecting a chromic acid-acid plating solution against a surface in the form of a free jet, and passing a current through said jet largely in excess of the current required for normal depositions on an area corresponding to the cross-sectional area of said jet.
  2. A method according to claim 1, wherein said solution is supplied to said jet at normal room temperature.
  3. A method according to claim 1 wherein a plating solution of a chromium type is projected with sufficient force against a cathode surface that large quantities of gas disengaged at the cathode surface are displaced whereby metal can be deposited from said solution onto said cathode surfaces.
- In witness whereof, I have hereunto signed my name.
- WALTER S. BOHLMAN.